

Feb. 10, 1942.

A. H. BURKHOLDER ET AL

2,272,182

METHOD OF PROCESSING THREAD OR THE LIKE

Filed May 3, 1938

3 Sheets-Sheet 1



FIG. 1



FIG. 3



FIG. 4

Inventors

ALDEN H. BURKHOLDER AND  
WALTER F. KNEBUSCH

by *Charles E. Herrstrom* Attorney

Feb. 10, 1942.

A. H. BURKHOLDER ET AL

2,272,182

METHOD OF PROCESSING THREAD OR THE LIKE

Filed May 3, 1938

3 Sheets-Sheet 2



Inventors

ALDEN H. BURKHOLDER AND  
WALTER F. KNEBUSCH

by *Charles E. Herstrom*  
Attorney

Feb. 10, 1942.

A. H. BURKHOLDER ET AL.

2,272,182

## METHOD OF PROCESSING THREAD OR THE LIKE

Filed May 3, 1938

3 Sheets-Sheet 3



FIG.13



FIG. 14



Fig. 15



FIG. 16

## Inventors

ALDEN H. BURKHOLDER AND  
WALTER F. KNEBUSCH

by Charles E. Herrstrom

Attorney

## UNITED STATES PATENT OFFICE

2,272,182

METHOD OF PROCESSING THREAD OR  
THE LIKE

Alden H. Burkholder, Cleveland, and Walter F. Knebusch, Rocky River, Ohio, assignors to Industrial Rayon Corporation, Cleveland, Ohio, a corporation of Delaware

Application May 3, 1938, Serial No. 205,678

6 Claims. (Cl. 18—54)

This invention relates to the processing of thread or the like and, more particularly, to methods of subjecting thread or the like to the action of processing liquid while it is continuously but temporarily stored in a plurality of generally helical turns on a thread-advancing, thread-storage device. While the invention provides great advantages in the processing of any kind of thread or the like, it may be employed to especial advantage in the liquid processing of artificial silk thread. The invention is particularly applicable to the type of liquid processing operation employed in the manufacture of viscose artificial silk thread by the so-called continuous method.

If a continuous process of the latter type employing one or more liquid processing steps is to be commercially successful, several conditions must be satisfied. In the first place, in order that the thread may be of commercially acceptable quality, it is necessary that the thread shall not be damaged as a result of the processing. It is likewise necessary that the thread shall be both thoroughly and uniformly acted upon by the processing liquid or liquids. Furthermore, if the process is to be commercially feasible, it is extremely important that the smallest possible amounts of processing liquids be employed to treat the thread.

The last-mentioned qualification arises out of the fact that in a commercial plant for the manufacture of viscose artificial silk thread it is necessary, in order to obtain the requisite commercial production, that several thousand threads be produced simultaneously. If excessive amounts of liquid are required to process each thread, the cost of the processing liquids becomes so high and the costs involved in conducting large quantities of processing liquids to and in the machines become so great as to render the process as a whole impracticable. This is particularly true in the manufacture of viscose artificial silk thread, which must be subjected to processing liquid at several different stages in the process of manufacture.

With these considerations in mind, it has long been recognized in the art that if viscose artificial silk thread is to be continuously processed, it must be subjected to the action of the processing liquids while stored in generally helical form on one or more thread-advancing thread store devices. It has been further appreciated that it is desirable that such thread-advancing thread store devices be self-threading; that is, that such devices should not require that each of the nu-

merous turns of thread be wound thereabout by hand. The reasons for these desiderata can be realized when it is understood that many thousands of such thread-advancing thread store devices are necessary in a single commercial plant.

Heretofore, when the thread has been subjected to liquid processing treatment on such devices, numerous difficulties have been encountered. Because in such devices the turns of thread are supported at spaced points, it has heretofore been thought necessary to have a relatively wide spacing of the turns, this more especially in order to prevent entangling of adjacent turns. However, even with such wide spacing of turns a great deal of difficulty has often been encountered. For example, the processing liquid has tended to cause individual turns to be washed out of position into contact with other turns; also, it has not infrequently happened that a globule of processing liquid clinging to two adjacent thread turns has tended, due to the surface tension of the processing liquid, to draw the turns together.

Where turns are thus displaced, they form a bundle on the thread-bearing periphery of the device in which bundle certain turns are disposed over or under adjacent turns and in which the filaments of adjacent turns are usually badly entangled. When, subsequently, the thread bundle so formed is discharged from the device, the entangled overwound or underwound turns tend to break, as do also the snagged filaments. As a result, the quality of the thread is considerably impaired, often sufficiently to render the thread useless for the purpose originally intended.

Moreover, because of the wide spacings heretofore employed, a large portion of the processing liquid has not adhered to the turns, but has merely dropped off between them. As a result, a large portion of the applied processing liquid has not served to process the thread, but has been wasted. In addition, because the processing liquid has generally been applied to the thread in one or more streams from a point or points above the respective thread-advancing thread store devices, the streams of processing liquid have necessarily been in contact with the thread in each turn for only the very short interval required to advance the turn therethrough. In some cases, not all of the thread in each turn has come into contact with the stream or streams of processing liquid, resulting in insufficiently processed portions of the thread.

All of the foregoing and numerous other difficulties are obviated by the present invention.

While according to the teachings of the invention the thread is subjected to processing liquid while stored on a rotating thread-advancing thread store device which serves to advance the thread lengthwise thereof in a plurality of generally helical turns, the conditions under which the thread is processed in accordance with the present invention are such that the processing liquid is caused to form a substantially continuous film over a substantial portion of the periphery of the thread-advancing, thread store device. Therefore, a number of turns of thread are completely enveloped in a thin layer of processing liquid, in consequence of which fact the thread may be much more thoroughly and uniformly processed than has heretofore been possible. Moreover, the thread may be effectively processed with the application thereto of a great deal less liquid than would otherwise be required.

In the drawings, in which are shown several forms of apparatus by means of which the invention may be practiced, Figure 1 is a perspective of a preferred form of such apparatus. Figure 2 is a side sectional elevation of a portion of said apparatus, parts being broken away to show the construction of the illustrated thread-advancing thread store device. Figure 3 is a front elevation of a portion of the apparatus of Figure 2, showing one of the thread-advancing thread store devices. Figure 4 is a plan sectional elevation of the preferred form of apparatus from line 4—4 of Figure 2.

Figure 5 is a diagrammatic elevation on a greatly enlarged scale showing in cross section two adjacent turns of thread disposed on a reel bar member. Figure 6 is a fragmentary plan of the turns of thread or the like of Figure 5. Figure 7 is a diagrammatic representation to the same scale as Figure 5, showing in cross section the filaments of adjacent turns of thread in the relation which they may assume when the thread is processed according to the present invention. Figure 8 is a fragmentary plan corresponding to Figure 7. Figure 9 is a diagrammatic representation on the same enlarged scale illustrating another arrangement which the filaments may assume showing in cross section the filaments along a bar member. Figure 10 is a fragmentary plan thereof. Figure 11 is another diagrammatic representation on the same enlarged scale showing in cross section the filaments in still another arrangement which may be obtained when the thread is being subjected to processing liquid according to the present invention. Figure 12 is a fragmentary plan corresponding to Figure 11.

Figure 13 is a side sectional elevation of a portion of another form of apparatus by means of which the invention may be practiced showing one of the thread-advancing thread store devices. Figure 14 is a corresponding front elevation. Figure 15 is a sectional elevation of a portion of still another form of apparatus by means of which the invention may be practiced. Figure 16 is a sectional elevation thereof from line 16—16 of Figure 15. In these and the other figures of the drawings, like reference characters refer to like parts throughout.

For convenience, the invention will be described in connection with the continuous processing of multiple filament viscose artificial silk thread on apparatus similar to that shown, described and claimed in copending application Serial No. 7,114 (Patent 2,225,642).

In such apparatus, thread 1 from a suitable source is passed in sequence to each of a plural-

ity of thread-advancing thread store devices 2 on each of which the thread is subjected to a processing treatment. The illustrated apparatus may be generally similar to that of the above-mentioned prior application in that the apparatus as a whole may comprise a plurality of downwardly extending series of thread-advancing thread store devices each of which operates on a single thread. Corresponding devices of such adjacent series may be disposed in corresponding positions longitudinally of the machine whereby advantages are provided in the construction of the apparatus and in the liquid supply and collecting systems.

The individual thread - advancing thread store devices preferably take the form of thread-advancing reels of the type shown, such reels operating on the same principle as the reel shown, claimed and described in copending application Serial No. 652,089 (Patent No. 2,210,914). The illustrated reels are, however, of cantilever form; that is, each is supported and driven from one end only. Each advances the thread toward the free end of the reel in a large number of closely spaced generally helical turns. Numerous benefits are provided by the cantilever construction of the reel, among them being ease of starting the thread on the reel, advantages in transferring the thread to the succeeding devices, etc.

Because of the cantilever construction of the reels, they can be disposed as shown in Figure 2 in stepped relation with the unobstructed end of each reel in apposite relation to the supported end of the succeeding reel. Numerous advantages are provided by such arrangement, among them the fact that the thread does not have to bend sharply in passing from one reel to another. As a result it is possible to avoid the stresses induced by sharp bending, which stresses would tend to injure the thread. Moreover, such a stepped arrangement of reels is advantageous in that the reels are readily accessible for operating purposes, as for starting the thread on the reels, for inspection and maintenance, etc.

The operation and construction of the illustrated reels will be explained in connection with Figures 2, 3 and 4.

As shown in these figures, each reel is made up of two rigid generally cylindrical reel members 4 and 5. Each reel member comprises a plurality of spaced longitudinally extending bar members disposed alternately with respect to those of the other member. Thus reel member 4, which may be termed the concentric member, has its periphery formed of a plurality of spaced parallel bar members 6 and is concentrically mounted on a drive shaft 7 journaled in a frame member 8. The other reel member 5, which may be termed the eccentric member, has a generally cylindrical periphery formed of a plurality of spaced longitudinally extending bar members 9 alternately disposed to the bar members 6 of reel member 4. Said reel member 5 is mounted for rotation about an axis offset from and inclined to that of reel member 4. The axes of the reel members are preferably disposed as shown in Figure 2; that is, inclined from the horizontal.

Concentric member 4 may be formed as shown with the bar members 6 formed on the periphery of a cylindrical body 11, in which case great rigidity is obtained. While said reel member 4 may be mounted on the drive shaft 7 in various manners, in that shown the generally cylindrical body 11 is concentrically mounted on a reduced portion of the drive shaft 7, being held

against a shoulder on said drive shaft by a cap-nut 12 threaded on the end of the drive shaft 7. The body 11 is provided with slots 13 at the rear end thereof, in which slots are disposed the projecting ends of a pin 14 disposed diametrically in said drive shaft, whereby the reel member 4 is caused to rotate with drive shaft 7.

In the illustrated embodiment, the eccentric reel member 5 is formed of a rigid cage-like member 15 having an internal annular rib 18 at the unsupported end of the reel which rib serves to reinforce the bar members 8 at said end. At the other end is an external annular rib 16 which serves to reinforce the bar members 8 and which also serves as means by which the cage-like member 15 is mounted on an annular member 17 which is journalled on frame member 8 for rotation about an axis disposed in the desired offset and inclined relation to that of the drive shaft 7. In the illustrated apparatus, the frame member 8 for each reel is mounted on the inclined beam 18 forming part of the frame of the apparatus.

The reel members may be made of some material resistant to the action of the processing liquids, while sealing means, such as a bellows-shaped rubber diaphragm 19, may be provided to seal the bearing means against entrance of processing liquid.

Rotation of the reel drive shaft 7 causes concentric member 4 fixed thereto to rotate, whereupon contact of the bar members 8 of concentric member 4 with the bar members 9 of eccentric member 5 causes said eccentric member to rotate at the same angular speed. During such rotation, the offset relation of the generally cylindrical reel members 4 and 5 causes the thread in each turn to be transferred from the bar members of one reel member to those of the other reel member. Simultaneously, the inclined relation of the reel members causes the thread to advance in a plurality of generally helical turns lengthwise of the reel. The magnitude of the inclination between the axes of the reel members, indicated by the angle  $\alpha$  in Figure 4, determines the pitch of the helical turns of thread; that is, the greater the angle  $\alpha$ , the greater is the pitch of the helical thread turns.

The reels may be driven by any suitable means; for example, from a drive shaft 21 disposed parallel to the inclined beam 18 and driving a plurality of reels in a processing series, one of the gears 22 mounted on said drive shaft meshing with a gear 23 mounted on each reel drive shaft 7.

In the embodiment of Figures 1 to 4, inclusive, processing liquid is applied to the thread stored on each reel from a tube 24 which is supplied with processing liquid from a conduit 25 extending longitudinally of the machine and serving corresponding reels in a horizontal series. The processing liquid is collected in a suitable collecting trough 26 extending beneath the reel, which trough may likewise serve a plurality of reels in a horizontal series. Therefore, each trough collects the liquid applied to the reel above it and also, by means of the reagent supply conduit formed integrally therewith, supplies processing liquid to the succeeding reel in the processing sequence. Each of said troughs is formed with a recessed portion 27 through which the thread passes from the reel above the trough to the succeeding reel, a suitable guide 28 being provided, if desired, to guide the thread onto the succeeding reel.

According to the present invention, the processing liquid is caused to form a continuous film or sheet of liquid in which the thread turns are contained and which preferably extends entirely around the reel over a substantial portion of the thread-bearing periphery thereof.

In order that the film of processing liquid may be formed and maintained it is necessary, for a given size of thread, that the thread turns be spaced considerably more closely than in the practices heretofore followed. The thread turns should be spaced closely enough, in fact, to permit the processing liquid adhering to adjacent thread turns to form a film therebetween. If the thread turns are too widely spaced, particularly with respect to the size of the thread, the distance between adjacent thread turns is too great to allow the film of processing liquid to be formed and maintained. Rather, under such circumstances the liquid adhering to the thread tends to cause the filaments in each thread turn to contract into a small cross sectional area. The effect of spacing of thread turns, number of filaments in the thread, and size of the thread can be better appreciated from a consideration of Figures 5 to 12, inclusive.

As shown by Figure 5, which represents a cross sectional view on a greatly enlarged scale of two adjacent thread turns supported by one of the

30 reel bar members, and by Figure 6, which represents a fragmentary plan elevation thereof, when the thread is being subjected to processing fluid under the conditions obtaining in the practices heretofore followed, no film of processing liquid is formed between adjacent thread turns. This arises because adjacent thread turns are so widely spaced that the processing liquid on the thread turns cannot form a film between adjacent turns. Rather, the filaments in each 40 thread are disposed in unitary bundles at spaced points along the bar members, the bundles of filaments being compact in cross section due to the fact that the surface tension of the liquid clinging to the filaments tends to draw them into a bundle of as small cross section as possible. The relatively great space heretofore employed between adjacent thread turns in proportion to the size of the thread, which wide space has 45 been thought necessary in the prior practices to prevent the filaments of adjacent thread turns from entangling, is also apparent from these figures.

50 Figures 7 to 12, inclusive, show the positions which may be assumed by the filaments in adjacent turns of thread when a film of processing liquid is formed according to the present invention.

55 As is apparent from these figures, the filaments of the thread turns are spread out into a thin layer extending completely around the reel, this because the surface tension of the processing liquid which is carried by the filaments causes the liquid to form a film between the filaments. As shown in Figures 7 and 8, for instance, under suitable conditions and particularly when the pitch of the advancing helix of thread and number and size of filaments are properly related, the filaments of adjacent thread turns will spread 60 into a single layer over the thread-bearing periphery of the reel. Figures 7 and 8 represent two adjacent turns of thread on the same scale as Figures 5 and 6. Under suitable conditions, as when the pitch of the advancing helix is greater 65 or the number of filaments is less than under 70 the conditions illustrated in Figures 7 and 8, ad-

jacent filaments will be more widely spaced than shown in these figures, so that the filaments do not contact with each other, as shown in Figures 9 and 10. The processing liquid adhering to the filaments, however, forms a continuous film covering all of the filaments.

Figures 11 and 12 illustrate an arrangement of the thread filaments which perhaps occurs more frequently in the processing of thread according to the present invention than do the arrangements of filaments illustrated in Figures 7 to 10, inclusive. Under the conditions illustrated in Figures 11 and 12, the filaments of adjacent turns are spread out into a layer which is more than a single filament in thickness. This condition occurs with thread of ordinary size when the thread turns are more closely spaced than in Figures 7 to 10, inclusive, or when the thread contains a larger number of filaments. For instance, when continuous bundles of filaments, such as are to be cut into staple fiber, each of which bundles contains hundreds or thousands of filaments, are continuously subjected to liquid processing treatment on reels according to the present invention, it is desirable to advance the bundles in a helix the pitch of which is small enough to cause the filaments in the turns to spread out into a layer two or more filaments in thickness. Due to the fact that the filaments are so spread out, the number of layers of filaments is much less than the number of layers in which the filaments would be disposed if the thread were processed according to the prior practices, as shown in Figures 5 and 6. This results in great advantages in processing, as will be hereinafter pointed out.

As previously explained, the spacing between the thread turns is determined in the case of the illustrated reel by the angle of inclination between the reel members, indicated, for example, by the angle  $a$  in Figure 4. With such a reel, very accurate control over the spacing of the thread turns can be obtained. Furthermore, the thread turns can be very accurately closely spaced. These advantages follow from the fact that the thread turns are advanced only by the rotation of rigid reel members about inclined axes and by no other moving parts between which there could be no lost motion.

For a reel of given diameter, the speed of rotation of the reel also plays a relatively important part in the formation and maintenance of the film of processing liquid. The speed of rotation of the reel should be high enough to cause the development of sufficient centrifugal force acting on the film to maintain the film; that is, the speed of rotation should not be so low that the processing liquid applied to the thread on the reel, as from a point above the reel, merely drops off the thread when at the upper portion of the reel. On the other hand, the speed of rotation of the reel should not be so high that the centrifugal force developed is great enough to throw off sufficient processing liquid from the film to destroy it. These factors provide the limits for the rotative speed of the reel; but between these limits the speeds may be varied to a considerable extent and satisfactory results still be obtained.

The number of bar members carrying the thread turns, the width of said bar members, and the spacing therebetween also influence to a certain extent the formation of the film of processing liquid.

The manner in which the processing liquid

is applied to the thread also affects the formation and maintenance of the film of processing liquid. In general, most satisfactory results are obtained when the liquid is applied to the thread on the reel from above the reel and substantially tangentially thereto, since if the processing liquid were to be applied to the thread in the reel in one or more substantially radial streams, the streams of processing liquid might 10 disturb the filaments or thread turns, causing them to entangle. Preferably, the processing liquid is applied against the direction of rotation of the reel, as shown, for instance, in Figures 1 to 4, inclusive, since thereby formation and 15 maintenance of the film of processing liquid are facilitated.

The amount of liquid which is applied to the thread should not be too little, else the film of processing liquid will not be formed due to the 20 fact that an insufficient quantity of liquid adheres to the thread. In such case, non-uniformity of the spacing of thread turns and discontinuities in the film of processing liquid will occur. On the other hand, the amount of 25 processing liquid which is applied to the thread should not be too great, since such excess processing liquid does not increase the effectiveness of the processing of the thread, but merely drops off into the trough 26.

As shown in Figures 1 to 4, inclusive, and in Figures 13 and 14, the reels are preferably inclined somewhat from the horizontal, the end at which the thread leaves the reel being higher than the end at which the thread starts on the 30 reel. When the reel is thus inclined, a very effective countercurrent flow of processing liquid is provided since the processing liquid may be applied to the elevated end of the reel and be caused to travel toward the lower end of the reel in the film of processing liquid. This makes for very efficient processing of the thread, since the thread which has just started on the reel is subjected to the action of processing liquid which has previously been used to treat other 35 portions of the thread, while the thread approaching the point at which it is to leave the reel is subjected to fresh processing liquid.

The amount of inclination of the reel from the horizontal influences the successful formation and maintenance of the film of processing liquid on the thread turns. If the amount of inclination is too great, the liquid will tend to run toward the lower end of the reel too rapidly and hence a film of processing liquid cannot be formed and maintained. If the amount of inclination is too small, the processing liquid will not travel entirely toward the lower end of the reel and hence a continuous film will be obtained only over a limited portion of the reel. 40 In general, the reel should be inclined only a very few degrees, the exact amount being dependent to a certain extent on other factors. The magnitude of the inclination is preferably 45 of the order indicated in the examples hereinafter given.

In connection with the processing of the thread under conditions in which a film of processing liquid is formed over the thread turns, the 50 exact amount by which the bar members of each reel member are retracted within the thread-bearing bar members of the other reel member is likewise important. If the amount by which the bar members are retracted is too great, the 55 film of processing liquid will break between the

thread turns and the retracted bar members. Rupture of the film of processing liquid may cause certain of the filaments, which, as has been stated, are spread out in a thin layer, to override the filaments of adjacent thread turns. When this occurs, the displaced filaments tend to break as the thread is unwound from the reel. Therefore it is important that the bar members of each set should not be retracted to too great an extent within such of the bar members of the other set as are carrying the thread, but should be withdrawn only sufficiently to permit the thread-advancing operation to take place.

The effect of the amount by which the bar members of each set are retracted within the other set forms the subject matter of copending application Serial No. 205,363.

In the preferred form of apparatus shown in Figures 1 to 4, inclusive, and to particularly good advantage in Figure 1, the thread 1 starts on each reel 2 at the supported end thereof and is advanced toward the free end of the reel, from which it is caused to leave the reel. The reel is inclined from the horizontal, the free end of the reel being higher than the supported end. The processing liquid is applied to the thread on the reel in a single stream 31 from the tube 24 above the reel, which tube may be a glass tube bent to the shape illustrated. The stream of processing liquid is directed downward on the thread windings at a point near the discharge end of the reel, the stream being directed against the direction of rotation and substantially tangentially to the reel.

In operation, the reel is rotated at an angular speed the rate of which is in part dependent upon the size of the reel and other factors, as will appear from the examples hereinafter given of actual operation according to the present invention. The thread turns are advanced in a helix of suitably small pitch dependent in part upon the size of the thread and other factors. Under such circumstances, as will be apparent from the hereinafter described examples, the processing liquid applied to the thread and adhering thereto forms a film between adjacent turns of thread due to the surface tension of the liquid. Due to the inclination of the reel, the processing liquid travels toward the lower end of the reel and the film of processing liquid is formed and maintained over the entire length of the thread winding on the reel.

As shown in Figures 1 and 2, because the processing liquid is applied substantially tangentially to the reel against the direction of rotation of the reel, a comparatively thick layer 32 of processing liquid is formed over a portion at least of the thread winding on the reel. The processing liquid in said layer tends to drop downward over the periphery of the reel, but said layer is maintained because the thread on the reel is moving upward in a clockwise direction. The formation of this layer of liquid, which may extend substantially along the entire length of the thread winding on the reel, is advantageous because it acts as a source of supply for the film of processing liquid along the length of the reel and since it conveys excess processing liquid which is not carried by the film toward the supported end of the reel.

When the processing liquid reaches the supported end of the reel; i. e., the end on which the thread starts, it can travel no farther, due to the fact that the bar members extend beyond the

end of the thread winding and cannot maintain the film. Therefore, the processing liquid leaves the reel at the end of the winding adjacent the supported end of the reel either in a more or less continuous stream as shown in Figures 1 to 4, inclusive, or in drops or masses of liquid, being collected in the collecting trough 26. Relatively little liquid is thrown off the reel by centrifugal force since in general the liquid collects into a mass which drops from the reel at the rear. An effective countercurrent flow of processing liquid is thus obtained, the thread being subjected to fresh processing liquid at the end of the reel from which it leaves the reel.

Due to the surface tension of the liquid, the filaments of the thread turns are spread out into a thin layer, as above illustrated, which layer is contained in and supports a film of processing liquid. In fact, during the processing of the thread and rotation of the reel, adjacent turns of thread are practically indistinguishable from each other along the length of the reel on which the film is formed. Indeed, as the reel rotates, the thread on the reel appears to consist of a thin layer of filaments, extending entirely around the reel and along its thread-bearing periphery, contained in a film or layer of liquid. However, when the thread reaches the free or discharge end of the reel, it may be withdrawn with no difficulty, since the filaments forming the thread are not entangled in adjacent thread turns.

While the reel is operating and the thread is being processed, adjacent thread turns are practically indistinguishable from each other, as above indicated; however, when the processing operation is being started, conditions are different. Reels of the illustrated type are self-threading; that is, in starting the thread on the reel it is only necessary to bring the wet thread into contact with the rotating reel, after which the thread will be advanced lengthwise of the reel in a plurality of generally helical turns. In the apparatus of Figures 1 to 4, inclusive, after the thread has been started on a reel and until the initial thread turns reach the stream of processing liquid at the discharge end of the reel, the filaments in each thread turn adhere to each other so that adjacent thread turns are clearly distinguishable from each other, being in general in the condition illustrated in Figures 5 and 6, though perhaps not so widely spaced.

However, when the thread turns approach the free end of the reel, the stream of processing liquid reaches the thread turns, with the result that the filaments spread as the film of processing liquid is formed during rotation of the reel. The film of processing liquid advances toward the lower end of the reel; i. e., the supported end of the reel in these figures, and the filaments of the thread turns spread as the film advances. Thus after the reel has become completely threaded up, the thread on the reel changes in a very short time from a state in which the thread turns are clearly distinguishable to a state in which the filaments are spread out and the thread turns are substantially indistinguishable. After the film has been thus formed, it is maintained while the thread is processed, as previously described.

While Figures 1 to 4, inclusive, illustrate a preferred form of apparatus by means of which the invention may be practiced, the arrangement shown therein is not the only one by means of which the results of the present invention may be obtained. As shown in the embodiments of Figures 13 and 14, for instance, the stream of proc-

essing liquid 31 from the tube 24 may be supplied substantially tangentially to the reel but in the same direction as the direction of rotation of the reel. Under these circumstances a film of processing liquid similar to that previously described will be formed and maintained over the thread windings. In the apparatus of Figures 13 and 14, as in the apparatus shown in Figures 1 to 4, inclusive, the processing liquid will travel in the film toward the lower or supported end of the reel and drop off into the collecting trough 26.

It is not necessary that the reel be inclined from the horizontal in order to cause the formation of the film of processing liquid over the reel. As shown in Figures 15 and 16, it is also possible to obtain a continuous film of processing liquid which extends entirely around a reel which has its axis horizontal. Under these circumstances, however, the effect of the inclination of the reel in aiding the formation of the film of processing liquid along the thread-bearing surface of the reel is absent.

In such circumstances, it is desirable, as in the apparatus of Figures 15 and 16, to provide a plurality of spaced streams 31a for distributing the liquid along the thread-bearing periphery of the reel. Each stream of liquid, impinging on the thread turns on the reel, tends to spread out and form a film of processing liquid due to the surface tension thereof, which film, during rotation of the reel, extends completely around the reel for at least a portion of the length of the thread-bearing periphery of the reel. The streams of processing liquid should be sufficiently closely spaced and should discharge in such amounts that the film formed by each stream merges with the adjacent film and thus forms a continuous film of processing liquid over the entire thread-bearing portion of the reel. Preferably, the streams of processing liquid should be directed substantially tangentially to the reel against the direction of rotation thereof because of the above-discussed advantages in the formation and maintenance of the film.

The spaced streams of liquid may be applied to the thread on the reel by various means. In the apparatus illustrated in Figures 15 and 16, the liquid is applied from a reagent distributor 33. Said distributor comprises a trough-like member 34 which is disposed below a hole 35 in the reagent supply conduit 25. One face of the trough-like member 34 of the reagent distributor 33 is provided with vertically extending grooves 36 in which are disposed weir notches or slots 37 extending through the wall of the trough-like member. By this means the processing liquid is caused to flow on the reel in a suitable number of streams of suitable magnitude to form a continuous film of processing liquid over the thread turns on the rotating reel. The liquid leaving the reel is collected in trough 26.

The following examples are illustrative of the conditions under which thread or the like may be continuously subjected to liquid processing treatment according to the present invention.

Very satisfactory results have been obtained when viscose artificial silk thread of 150 denier and 40 filament is subjected to liquid processing treatment on a cantilever reel of the illustrated type forming part of apparatus of the general type shown in Figures 1 to 4, inclusive. The thread-bearing portion of each reel member is 5" in diameter, each reel member comprising 14 bar members, the total length of the portion of the reel covered by thread winding being 4".

The bar members of the concentric reel member are  $\frac{1}{4}$ " wide, while those of the eccentric reel member are  $\frac{1}{8}$ " wide. The reel members rotate about axes which are offset from each other in parallel planes, the amount of such offset being very close to  $\frac{1}{2}$ ". The reel is inclined from the horizontal with its unsupported end higher than its supported end, the amount of inclination being  $\frac{1}{8}$  inch per inch or  $3^\circ 35'$ . The thread is, of course, advanced toward the free end of the reel.

Processing liquid is applied to the thread on the reel in a single stream at the discharge end of the reel, the stream being directed against the direction of rotation of the reel and substantially tangentially thereto, substantially as shown in Figures 1 to 4, inclusive. Approximately 270 c. c. of processing liquid per minute are thus supplied to the thread on the reel through an orifice .075" in diameter in the tube 24. It is desirable that the angle of inclination of the reel members be such that the number of turns of thread will be not fewer than 20 per inch but satisfactory results will still be obtained if as many as 60 turns per inch are used, but preferably between 27 and 40 turns per inch are employed.

As an example, a film of processing liquid of the type to which the present invention is directed can be obtained within the above-indicated pitch range if the processing liquid is washing water. The reel is rotated at 170 R. P. M., although a somewhat lower speed may be employed, and good results are obtained up to 200 R. P. M. With a reel of the above size, the centrifugal force acting on the film of processing liquid appears to be too great at speeds substantially above 200 R. P. M. When thread of the above-indicated size is processed according to the above conditions, a continuous film of processing liquid is formed which extends completely around the reel over the entire length of the thread windings on the reel. The thread is thoroughly and uniformly processed and has highly uniform characteristics throughout its entire length.

Effective processing is also obtained when a bundle of viscose filaments of 5,000 denier containing 1,700 filaments, such as is employed in making staple fiber, is subjected to liquid processing treatment on a cantilever reel operating on the same principle as the reel illustrated. The thread-bearing portion of each reel member of such reel is 17" in diameter and the portion of the reel covered by the thread winding is 7" long. Each reel member comprises 30 bars, each  $\frac{1}{2}$ " wide and the reel members rotate about axes which are disposed in parallel planes offset  $\frac{1}{4}$ ". The reel is inclined from the horizontal with its free end higher than its discharge end, the inclination of the reel being  $\frac{1}{8}$ " per inch, or  $3^\circ 35'$ , the thread being advanced toward the free end of the reel.

A single stream of processing liquid is applied from a tube to the thread on the reel at a point near the upper portion of the reel and near the free end thereof, the stream being directed tangentially of the reel in the direction of rotation thereof. The stream of processing liquid supplies 5,000 c. c. of processing liquid per minute, through an orifice .315" in diameter in the reagent tube, to the thread on the reel. The processing liquid is one of the liquids employed in processing viscose thread or the like. The angle of inclination between the reel members is such that the bundle of filaments is stored in an ad-

vancing helix having 4 turns per inch, the reel being rotated at 66 R. P. M.

Under the above conditions a continuous film of processing liquid, which extends completely around the reel and longitudinally thereof over the entire length of the thread windings on the reel, is formed, the filaments being spread out into a thin layer contained in the film of processing liquid.

Because according to the present invention the filaments of the turns of thread are spread out into a thin layer which is one or at most only a few filaments thick, the processing medium may reach all parts of all filaments much more readily than is possible when the filaments are not spread into a thin layer but are piled up as shown in Figures 5 and 6. When the filaments are disposed as shown in said figures, which illustrate the condition occurring in the prior practice, it is extremely difficult for the processing liquid to reach the innermost filaments and hence non-uniform processing often results. Moreover, since according to the present invention the filaments in their spread condition are contained in a layer of processing liquid which extends entirely around the reel and contacts with all parts of the filaments, the thread is more uniformly and more thoroughly processed than heretofore possible. Therefore thread of a higher quality may be produced according to the present invention than is possible according to the thread-processing practices heretofore employed.

According to the present invention, furthermore, it is possible to cause substantially all of the processing liquid applied to the thread to adhere to the turns of thread in the form of a sheet or film of processing liquid. Very little, if any, excess liquid need be applied to the thread, particularly if the thread is processed by means of apparatus similar to the type shown in Figures 1 to 4, inclusive. Consequently, very efficient processing of the thread is made possible by the present invention and the amount of processing liquid which it is necessary to apply to the thread is greatly reduced as compared with the amount necessary in prior practices.

Actual tests have revealed that when 150 denier 40 filament viscose artificial silk thread is processed on a reel of the illustrated type having reel members 5" in diameter under the conditions of the prior practices, no film of processing liquid being formed, more than three times as much washing water is necessary to thoroughly wash the thread as is required when thread of the same kind is processed on a reel of the same size according to the present invention. In this respect the present invention results in reduced production costs, both from the standpoint of the liquid consumed and since the costs involved in transporting and pumping the liquids for the large number of thread-advancing, thread-storage devices used in commercial apparatus are considerably reduced. Thus, smaller conduits and other liquid-handling equipment may be employed with resultant reduced construction costs.

Numerous other advantages of the invention will be apparent.

The above-illustrated forms of apparatus by means of which the invention may be practiced and the above-described examples of the present invention are purely illustrative. Thus, under suitable conditions, other types of thread store devices than that illustrated may be employed. Various modifications may be made in the illus-

trated apparatus without departing from the spirit of the present invention. The term "thread or the like" in the appended claims is intended to include all materials which may be subjected to liquid processing treatment according to the present invention.

It is intended that the patent shall cover, by suitable expression in the appended claims, whatever features of patentable novelty reside in the invention.

What is claimed is:

1. The method of subjecting thread or the like to the action of processing liquid which includes advancing the thread or the like in the form of a traveling helix characterized by a large number of turns individually supported at spaced points; applying the processing liquid to the thread or the like at one end of the helix, the turns of thread or the like at each end being sufficiently close to one another to permit the processing liquid to form a continuous film extending entirely around the helix; and causing the processing liquid to travel lengthwise of the helix, whereby the film of processing liquid so formed is caused to envelop a substantial portion of the helix.

2. The method of subjecting thread or the like to the action of processing liquid which includes applying the processing liquid to the thread or the like; advancing the thread or the like in the meanwhile in the form of a travelling helix characterized by a large number of turns individually supported at spaced points; and disposing the turns in said helix in sufficiently close relation to one another so that the processing liquid applied to the thread or the like extends between adjacent turns to form a continuous film of processing liquid extending over at least a portion of the periphery defined by said turns.

3. The method of subjecting thread or the like to the action of processing liquid which includes applying the processing liquid to the thread or the like as it is advanced in the form of a travelling helix characterized by a large number of turns individually supported at spaced points which turns are sufficiently close to one another to permit the processing liquid to form a continuous film extending entirely around the helix, meanwhile rotating the helix at a speed sufficient to enable the resulting centrifugal force to assist in maintaining the film.

4. The method of subjecting thread or the like to the action of processing liquid which includes applying the processing liquid substantially tangentially to the thread or the like, the thread or the like being advanced in the meanwhile in the form of a travelling helix characterized by a large number of closely spaced turns individually supported at spaced points which turns are sufficiently close to one another to permit the processing liquid to form a continuous film extending entirely around and for a substantial distance lengthwise of the helix.

5. The method of subjecting thread or the like to the action of processing liquid which includes advancing the thread or the like in the form of a travelling helix characterized by a large number of turns individually supported at spaced points which turns are sufficiently close to one another to permit the processing liquid to form a continuous film extending entirely around the helix, meanwhile applying the processing liquid to the thread or the like in a plurality of streams which are sufficiently closely spaced to cause ad-

acent streams to merge into a single film enveloping a substantial portion of the helix.

6. The method of subjecting thread or the like to the action of processing liquid which includes advancing the thread or the like in the form of a travelling helix with its axis of rotation at an angle to the horizontal characterized by a large number of turns individually supported at spaced

points which turns are sufficiently close to one another to permit the processing liquid to form a continuous film extending entirely around the helix, meanwhile applying the processing liquid toward the higher end of the helix.

5

ALDEN H. BURKHOLDER.  
WALTER F. KNEBUSCH.